

## UNITED STATES PATENT OFFICE

2,300,589

## ANIMALIZING CELLULOSEC FIBERS

Johannes Nelles, Leverkusen-Schlebusch, and Otto Bayer, Leverkusen I. G.-Werk, Germany, assignors, by mesne assignments, to General Aniline & Film Corporation, New York, N. Y., a corporation of Delaware

No Drawing. Application August 15, 1939, Serial No. 290,220. In Germany August 23, 1938

5 Claims. (Cl. 106—164)

The present invention relates to processes of increasing the affinity of cellulosic fibers towards wool dyestuffs, to the fibers so treated and to products suitable for the said processes.

It is known that the affinity of cellulosic fibers for acid wool dyestuffs can be increased by incorporating therewith substances of basic nature. Since thereby the cellulosic fibers, as far as dyeing is concerned, become more or less similar to animal fibers, such substances are commonly called "animalizing agents." Very suitable animalizing agents are, for instance, high molecular organic compounds containing basic groups, especially nitrogen, the high molecular character of which is caused by the presence of high molecular aliphatic radicals or by condensation or polymerization of low molecular basic compounds. It is also known that animalizing agents should be insoluble or difficultly soluble in water, in order not to be removed from the fibers by wet treatments. In view of their insolubility in water and aqueous liquids, animalizing agents were hitherto applied to the fibers or added to spinning solutions of artificial fibers in the form of solutions in organic solvents or in the form of aqueous dispersions.

We have now found an improvement in the art of animalizing which consists in employing such animalizing agents which, due to the presence of at least one sulfonamido group in their molecule, are soluble in alkali lyes. With the aid of these new animalizing agents it is now possible, for instance, to manufacture artificial fibers from viscose spinning solutions containing the animalizing agent homogeneously dissolved therein. Thereby the production of animalized artificial fibers is very much simplified because it is no longer necessary to prepare special solutions or dispersions of the animalizing agent and to apply such solutions or dispersions in special working steps to the material; also the disturbances are avoided which often occurred by obstruction of pipes or nozzles of the spinning apparatus, when dispersions of an animalizing agent were added to the spinning solution. Furthermore, an animalizing agent which is soluble in the spinning solution, can be more easily and homogeneously distributed throughout the fiber than a pulverized and dispersed insoluble agent.

The animalizing agents to be used according to our invention may be of various chemical structure. What they have in common are (1) the common characteristics of all animalizing agents, i. e. they are high molecular, water insol-

uble basic substances, which increase the affinity of cellulosic fiber treated therewith to acid wool dyestuffs; and (2) they contain one or more sulfonamido groups by which they are rendered soluble in alkali lyes, for instance, in caustic soda lye. As such animalizing agents there may be mentioned, for example, reaction products from aliphatic polyamines with arylsulfoethylenimides reaction products of chloroparaffinesulfon chlorides obtainable according to the U. S. Patent No. 2,046,090, with ammonia or ethylenediamine, condensation products of benzylchloride-p-sulfochloride with di- and polyamines, condensation products of naphthalene- and di-phenyl-poly-( $\beta$ -chloroethylsulfamide) with amines, reaction products of polystyrenesulfochloride with asymmetric dialkylethylenediamine, the formaldehyde condensation products of naphthalene-tri - (as - diethylethylenediaminesulfamide), and many others.

Our invention is furthermore illustrated by the following examples, the parts being by weight, if not otherwise stated:

Example 1

7.5% of a reaction product from polyethyleneimine and benzenesulfoethylenimide, (prepared according to Example 10 of the U. S. Patent No. 2,233,296 of Nelles et al, issued February 25, 1941), calculated on the weight of the cellulose, are dissolved in a small quantity of caustic soda lye and stirred into a viscose spinning solution. The solution is then worked up into viscose staple fibers as usual. The fibers so obtained have good affinity for acid wool dyestuffs and may be dyed alone or mixed with wool fibers, for instance, with Supranolbrillantred B (compare Schultz, Dyestuff Tables, vol. 2, 1932, p. 204), Anthralaneblue G (compare l. c., 1st supplemental vol., 1934, p. 68), Diamondblack P2B (compare l. c., vol 1, 1931, p. 104). Very level dyeings of good fastness to wet treatments are obtained.

Example 2

To a reaction product according to Example 10 of U. S. Patent No. 2,233,296 from 43 g. polyethyleneimine and 93 g. benzenesulfoethylenimide in about 300 ccm. chloroform, there are dropped 60 g. phenylisocyanate at 30-40° C. The solution is refluxed for 2 hours. After distillation of the solvent, a tough, nearly colorless resin is obtained which, by dissolving in dilute aqueous alkali, filtering and precipitating with

dilute acetic acid, can be freed from small quantities of alkali-insoluble products.

12% of this alkali-soluble animalizing agent are added to a viscose spinning solution which is worked up as usual. The fibers so obtained are dyed, alone or in mixture with animal fibers, by acid wool dyestuffs in very fast shades.

*Example 3*

Paraffine is treated with sulfur dioxide and chlorine according to the method described in U. S. Patent No. 2,046,090, until the chlorine content of the resulting product is about 38%. 300 parts of this product are heated for 10 hours to 115-120° C. with 270 parts ethylenediamine (78%) in 150 parts butyl alcohol, similarly as described in the French Patent No. 709,626.

7% of the resulting animalizing agent, calculated on the weight of the cellulose, dissolved in aqueous alkali are incorporated with a viscose staple fiber spinning solution. Fibers obtained therefrom are well dyed by acid wool dyestuffs.

*Example 4*

p-Aminobenzenesulfoethyleneimide (melting point 129-130° C.) is prepared according to Gabriel, Ber. d. deutsch. chem. Ges. 28, page 2933 by reacting p-acetylaminobenzenesulfochloride with ethyleneimine and saponifying with aqueous alkali. By heating the imide for several hours to 100° C., a polymeric, infusible, colorless polyamide is obtained which is soluble in dilute aqueous alkali.

4% of this product, dissolved in aqueous alkali, are added to a viscose spinning solution. The fibers obtained therefrom in the usual manner are of mat, wool-like appearance. They are easily dyed by acid wool dyestuffs, and the dyeings are of good fastness.

*Example 5*

184 g. cyanuric chloride are dissolved in 1 l. of warm acetone; the solution is stirred into an iced solution of 172 g. m-aminobenzenesulfamide in 750 ccm. acetone. The temperature is kept below +20° C. by adding ice, if necessary. The mixture is then acidified by adding sodium acetate and, after stirring for 2 hours, the resulting nearly colorless powder is filtered off and dried. It has a decomposition point above 300° C. and is of the probable formula:



96 g. thereof are stirred with 300 ccm. hexahydrodiethylaniline; into the mixture, 43.5 g. di-( $\gamma$ -aminopropyl)-methylamine are dropped at 20-30° C. After stirring for several hours at room temperature, the temperature is slowly raised to 80° C. and kept at that value for some hours. After cooling the solid reaction product is isolated and dried. It is a light powder being well soluble in dilute aqueous alkali.

10% of this product, dissolved in aqueous alkali, are stirred into a viscose spinning solution which is worked up as usual. The fibers obtained therefrom are well dyed by acid wool dyestuffs, for instance those mentioned in Example 1. Good tone-in-tone dyeings are obtained on mixed viscose-wool material in most cases.

We claim:

1. Process for increasing the affinity of cellulosic fibers towards acid wool dyestuffs which comprises incorporating with the fibers high-molecular weight, water-insoluble, alkali-soluble sulfonamides containing in addition to the nitrogen of the sulfamide groups, basic nitrogen atoms.

2. Process for increasing the affinity of artificial cellulosic fibers towards acid wool dyestuffs which comprises incorporating high-molecular weight, water-insoluble, alkali-soluble sulfonamides containing in addition to the nitrogen of the sulfamide groups, basic nitrogen atoms, with an alkaline cellulose solution and precipitating the fibers from said solution.

3. Process for increasing the affinity of artificial cellulosic fibers towards acid wool dyestuffs which comprises incorporating high-molecular weight, water-insoluble, alkali-soluble sulfonamides containing in addition to the nitrogen of the sulfamide groups, basic nitrogen atoms with a viscose spinning solution.

4. Cellulosic fibers having increased affinity towards acid wool dyestuffs, said fibers having incorporated therewith high-molecular weight, water-insoluble, alkali-soluble sulfonamides containing in addition to the nitrogen of the sulfamide groups, basic nitrogen atoms.

5. Viscose artificial fibers having increased affinity towards acid wool dyestuffs, said fibers having incorporated therewith high-molecular weight, water-insoluble, alkali-soluble sulfonamides containing in addition to the nitrogen of the sulfamide groups, basic nitrogen atoms.

JOHANNES NELLES.  
OTTO BAYER.